

June 4, 1935.

H. W. GRAHAM ET AL

2,003,710

METAL BODY RESISTANT TO FLUCTUATING STRESSES

Filed March 28, 1933



Patented June 4, 1935

2,003,710

# UNITED STATES PATENT OFFICE

2,003,710

## METAL BODY RESISTANT TO FLUCTUATING STRESSES

Herbert W. Graham and Samuel L. Case, Pittsburgh, Pa., assignors to Jones & Laughlin Steel Corporation, Pittsburgh, Pa., a corporation of Pennsylvania

Application March 28, 1933, Serial No. 663,155

5 Claims. (Cl. 285—146)

This invention relates to metal bodies resistant to fluctuating stresses and is hereby particularly described as applied to a drill pipe, although it has numerous other applications:

- 5 To take the example stated, drill pipes are subjected to severe and continuing fluctuating stresses, and in practice they frequently fail prematurely. The failure is highly objectionable not only because of the shortened life of the drill 10 pipe but also because it often takes place while the string of drill pipe is in the ground, frequently causing lost time and considerable expense for fishing. The threads constitute relatively sharp changes in surface configuration of the drill pipe 15 and it has been observed that failures of bodies subjected to fluctuating stresses are generally initiated at such point.

We have found that these defects may be overcome by making the body of steel having special 20 characteristics, and subjecting it, particularly in those portions where failure is most likely to occur, to a special treatment; which we have found greatly enhances the life of the article.

We use a non-aging steel which may be obtained, for example, by adding aluminum to the 25 steel in the amount of one to three pounds per ton; or an equivalent amount of an iron-aluminum alloy may be added. If desired, more aluminum may be added, but it will be found that five 30 pounds per ton will probably be sufficient in any case. This steel is processed in the usual way and the article is made therefrom. It is then subjected to cold work. This may be done by cutting the thread and thereafter subjecting it to the 35 action of a rolling or burnishing tool. On a drill pipe, for example, the tool may be used to apply cold work in an amount sufficient to reduce the diameter of the thread slightly, say about one-thousandth of an inch. It will be found that by 40 making the article of non-aging steel and subjecting it to cold work its qualities of resistance to fluctuating stress are greatly enhanced.

The accompanying figure of drawing illustrates 45 part of a string of drill pipes. Each drill pipe has a body 2 and thickened end portions 3 ex-

teriorly threaded as at 4 to accommodate couplings 5. On the drawing we have indicated the zone of cold work as extending over the threads. It will be understood that the couplings may be likewise cold worked and that if desired the cold working may extend over the entire article or over other selected parts thereof. 5

We have described a present preferred embodiment of our invention. It will be understood, however, that this is by way of illustration only 10 and that it may be otherwise embodied or practiced within the scope of the following claims.

We claim:

1. As a new manufacture, a drill pipe made of substantially non-aging steel, the drill pipe being 15 in the form of a hollow tube having a thickened end portion, which thickened end portion is threaded, the threaded portion at least being cold worked.
2. As a new manufacture, a drill pipe made 20 of substantially non-aging steel, the drill pipe being in the form of a hollow tube having a thickened end portion, which thickened end portion is threaded, the threaded portion at least being cold worked, and a coupling threaded to engage said 25 end portion of the drill pipe, the coupling being made of substantially non-aging steel and being cold worked.
3. As a new manufacture, a metal body 30 resistant to fluctuating stresses, the body being made of non-aging steel and having at least a portion thereof of enhanced resistance to fluctuating stress, said portion being cold worked.
4. As a new manufacture, drill pipe made of 35 substantially non-aging steel resistant to fluctuating stresses, at least a portion thereof being of enhanced resistance to fluctuating stress, said portion being cold worked.
5. As a new manufacture, a drill pipe made of 40 substantially non-aging steel resistant to fluctuating stresses, the drill pipe having a threaded end portion of enhanced resistance to fluctuating stress, said end portion being cold worked.

HERBERT W. GRAHAM.

SAMUEL L. CASE.

45